

## UNITED STATES PATENT OFFICE

FRANK W. ANDREWS, OF DAYTON, OHIO, ASSIGNOR, BY MESNE ASSIGNMENTS, TO  
FRIGIDAIRE CORPORATION, A CORPORATION OF DELAWARE

## ALLOYS

No Drawing.

Application filed April 28, 1927. Serial No. 187,353.

This invention relates to compositions of matter, particularly to alloys designed to be used for gaskets, packing material and the like.

5 One of the objects of the invention is to provide a metal which is sufficiently plastic to flow under moderate pressures so as to conform to irregularities in surfaces with which it is in contact. It is also an object of 10 the invention to provide a metal having the above characteristics which has a coefficient of thermal expansion close to that of the parts with which it is to be used.

Further objects and advantages of the 15 present invention will be apparent from the following description.

In constructing machinery having rotating parts whose bearings must be sealed against the passage of gas, for example compressors used in refrigerating apparatus, considerable difficulty has been encountered in packing the stuffing box which ordinarily surrounds the rotating shaft. My invention 20 contemplates a metallic packing which, due to its plasticity, can be made to conform accurately to the shape of parts of machinery so as to form a gas-tight seal and which, due to its coefficient of expansion, maintains such sealing contact thruout the variations 25 in temperature encountered in the operation of such machinery.

In the example mentioned, the machine parts are ordinarily made of cast iron and steel, metals having coefficients of expansion 30 sufficiently near each other to be considered the same thruout the temperature range under consideration. It is therefore important that the coefficient of expansion of the packing be substantially or approximately the same as 35 that of iron or steel. For if the packing metal expands at a widely differing rate, it will, as the temperature rises, either recede from the parts to cause leaks, or expand into such tight contact as to produce excessive friction, which may stop the machinery, if of 40 small power, or injure the parts through over-heating.

I have discovered that alloys containing 45 from 90% to 95% lead and the rest either 50 tin and bismuth, or tin, bismuth and anti-

mony, are well adapted to the purposes above described. Such alloys are sufficiently plastic to meet the requirements of gaskets and packing glands and their coefficients of expansion are sufficiently near the coefficients of cast iron 55 and the various steels with which they will be used. The coefficient of expansion may be varied to suit requirements by slightly varying the proportions of the constituent metals. For example I find that an alloy of 95 parts 60 lead, 3 parts bismuth, and 2 parts tin has a coefficient of expansion corresponding to that of steel such as ordinarily used for compressor shafts and that these proportions may be varied slightly without materially effecting 65 the result. The lead, being greatly in excess of the other components, can be varied to a greater extent without materially changing the result.

As particular examples of the component 70 elements of which I may make my alloy, and their proportions, I mention the following:

## Example 1

|         |       |             |    |
|---------|-------|-------------|----|
| Lead    | ----- | 90-96 parts | 75 |
| Tin     | ----- | 1-3 parts   |    |
| Bismuth | ----- | 2-4 parts   |    |

## Example 2

|          |       |             |    |
|----------|-------|-------------|----|
| Lead     | ----- | 90-96 parts | 80 |
| Tin      | ----- | 4-6 parts   |    |
| Bismuth  | ----- | 1-3 parts   |    |
| Antimony | ----- | 1-3 parts   |    |

I claim as my invention:

A plastic metallic packing composition having coefficient of expansion approximating that of cast iron and steel and consisting of lead, tin and bismuth in the following proportions:

|         |       |                |    |
|---------|-------|----------------|----|
| Lead    | ----- | 90 to 96 parts | 90 |
| Tin     | ----- | 1 to 3 parts   |    |
| Bismuth | ----- | 2 to 4 parts   |    |

In testimony whereof I hereto affix my signature.

FRANK W. ANDREWS.